

## UNITED STATES PATENT OFFICE.

NOAK VICTOR HYBINETTE, OF NEW YORK, N. Y.

## ALLOY, ETC.

No Drawing.

Application filed October 12, 1921. Serial No. 507,331.

This invention relates to improvements in nickel alloys which are non-corrodible and which have a resistance to acids and to a moist atmosphere comparable with or greater than that of pure nickel, and which are also soft and ductile so that they can be worked hot and cold by rolling, drawing, pressing, spinning, stamping, welding, etc. The alloys of the present invention are particularly adapted for such purposes as cooking utensils, condenser and boiler tubes, sheet nickel for tanks, etc. The invention includes improvements in the new alloys themselves as well as articles made therefrom.

It is known that nickel mixes or alloys with iron in all proportions to a solid solution, but such alloys, without further admixture, are not well adapted for use for the purposes mentioned. In a co-pending application, Serial No. 489,099, I have described improved alloys containing, in addition to nickel and iron, small and regulated amounts of other alloying metals and deoxidizers which give to the alloys the desired properties.

The object of the present invention is to further improve these soft ductile iron-nickel alloys so that their noncorrosiveness will even exceed that of pure nickel.

It is known that larger quantities of chromium will increase the resistance to acids, but I have found that such increase of over 5% chromium is insignificant compared with the drawbacks. The resistance against nitric acid may be slightly improved by using 10-15% chromium instead of 5%, but resistance to other chemicals is still less.

I add copper, tungsten and molybdenum; one or two, or all in combination.

In addition to the constituents mentioned in said application, copper may be added to the alloy in amounts of 3 to 5% without any bad effect from segregation, while the resistance against sulfuric acid is perceptibly increased.

If tungsten, and particularly if molybdenum, or both, in amounts of 1 to 5% of each, are added, the ductility is somewhat decreased, but the resistance against acids increases to the highest degree that can be obtained, so far as I am aware, in a soft, easily worked ferrous alloy. The alloys have such remarkable acid resistance that the difference between an iron-free alloy and one

with 2½ to 3 parts of iron to 1 part of nickel is relatively small and greater than of pure nickel. If a larger proportion of chromium is used instead of or in connection with molybdenum or tungsten, or copper, similar results are not obtained, and the metal becomes much harder. I therefore consider it important that none of the additions to the iron-nickel alloy should amount to above 5% or thereabouts.

The addition of the various metals need not exceed the following amounts, namely, 2% manganese, 3 to 5% chromium, 5% copper, 2% tungsten, and 1% molybdenum, as increased additions do not appear to be correspondingly advantageous.

The presence of vanadium, titanium, zirconium, etc. may not be objectionable but even beneficial in small amounts. The presence of copper in too large amounts may be ob-

jectionable on account of segregations, poisonous or galvanic action, etc. and it will be understood that copper may be omitted from the alloys, although its presence is unobjectionable for many purposes and it is advan-

tageous when present in small amounts to make the alloy softer and more acid resistant. The addition of copper makes possible the use of a copper-nickel product made direct from copper-nickel ore, thus enabling the

nickel to be directly introduced in this way instead of in the form of pure nickel. In many cases the copper may therefore advantageously be used even to the extent of say 10%, and particularly when at the same time the nickel contents are high, because the more iron the more chance for segregation of copper; but nickel helps against segre-

gation.

If the proportion of nickel is above 30%, and chromium, tungsten or molybdenum with or without copper are used to in the neighborhood of 5% each, the alloy becomes heat resisting, and is as such preferable to those already known, it being more malleable and easily drawn into wire.

It will thus be seen that the alloys of the present invention contain varying amounts of nickel and iron, and that the proportions of nickel and iron can be varied and regulated in accordance with the use for which the alloy is intended. In addition to the iron and nickel, and independent of their proportions to each other, I also add about 2% of manganese and 3 to 5% of chromium,

and may also introduce copper in some cases up to about 10%. All of the alloys are preferably deoxidized with manganese aluminum and magnesium for better ductility. For 5 very exacting requirements of non-corrodability, tungsten, molybdenum, are added in small quantities.

The present invention makes it possible to produce an alloy having strength, ductility, 10 resistance to corrosion, and appearance comparable to or even better than possessed by pure nickel, while the expense of the alloy is very greatly reduced as compared with that of pure nickel. The regulation and 15 control of the composition of the alloys and of the resulting properties makes it possible to produce alloys for various purposes, such as boiler tubes, condenser tubes, cooking utensils, roofing plates, chemical apparatus. 20 table ware, etc.

The following alloys are examples of an alloy which can be produced at moderate expense, and which has properties of strength, ductility and non-corrodability 25 fully comparable with those of pure nickel.

|       | Per cent | Per cent |
|-------|----------|----------|
| Fe.   | 60       | 60       |
| Ni    | 20       | 30       |
| Cu    | 10       | 0        |
| 30 Mn | 2        | 2        |
| Cr    | 3        | 3        |
| W     | 2        | 2        |
| Mo    | 1        | 1        |
| C     | 0.3      | 0.3      |
| 35 Si | 0.2      | 0.2      |
| Al    | 0.1      | 0.1      |
| Mg    | 0.05     | 0.05     |

In making the alloys, small amounts of 40 hardening agents and deoxidizing ingredients may be added, such as carbon, silicon, vanadium, titanium, zirconium, cerium, etc., but in general there appears to be little if any advantage in their use over aluminum 45 and magnesium, and for soft, ductile alloys they should be omitted or kept as low as economically possible. Carbon and silicon

may, however, be added in quantities up to 2% each to facilitate the casting of the alloy into intricate shapes of acid-resisting receptacles or structures, in which case, however, copper may have to be correspondingly reduced or even omitted so as not to cause segregation.

I claim:—

1. An alloy consisting mainly of nickel and iron and containing at least two-and-one-half times as much iron as nickel, said alloy also containing chromium, tungsten and molybdenum in substantial amounts not 60 exceeding about 8% in the aggregate, and a small amount of manganese.

2. An alloy consisting mainly of nickel and iron and containing at least two-and-one-half times as much iron as nickel, said alloy 65 containing chromium, tungsten, molybdenum and manganese in substantial amounts not exceeding about 8% in the aggregate, and copper in an amount not over about ten per cent.

3. An alloy consisting mainly of nickel and iron and containing at least two-and-one-half times as much iron as nickel, said alloy also containing chromium, tungsten and molybdenum in substantial amounts not 70 exceeding about 8% in the aggregate and copper in an amount not over about 10%.

4. An alloy consisting mainly of nickel and iron and containing at least two-and-one-half times as much iron as nickel, said 80 alloy also containing chromium, tungsten and molybdenum in substantial amounts not exceeding about 8% in the aggregate and also 3-5% of copper.

5. An alloy consisting mainly of nickel and iron and containing at least two and one-half times as much iron as nickel, said alloy also containing chromium, tungsten and molybdenum in substantial amounts not 85 exceeding about eight percent in the aggregate.

In testimony whereof I affix my signature.

NOAK VICTOR HYBINETTE.